

Feb. 16, 1954

E. CLARK

2,669,599

STORAGE BATTERY PLATE SEPARATOR

Filed Sept. 19, 1952

FIG. 1



FIG. 2



INVENTOR

EDWARD CLARK,

Myron P. Laughlin

ATTORNEY

## UNITED STATES PATENT OFFICE

2,669,599

## STORAGE BATTERY PLATE SEPARATOR

Edward Clark, Chicago, Ill.

Application September 19, 1952, Serial No. 310,478

6 Claims. (Cl. 136—145)

1

This invention relates to storage battery separators and more particularly to means for constructing and repairing such separators at reduced cost and increased effectiveness. Heretofore it has been usual to construct such separators of wood and in the preparation of such wood and separators, it has been essential that the natural acids and certain other deleterious elements be extracted through alkaline baths, steam treatment and the like which not only consumed time and materials, but often resulted in the destruction of the wood fibers and bonds and indeed prevented the use of certain woods altogether.

The herein disclosed process, material and apparatus eliminates these preparation steps and so provides for the protection of the separator material while in use that oxidation and charring is entirely eliminated. It thus permits the use of any wood or other material having sufficient mechanical strength when supplemented by my invention, and at the same time, completely eliminates costly special machinery and elaborate processes while completely neutralizing any defects which the natural material may have, or which elements absorbed by the wood might introduce.

It is a further purpose of this invention to provide a separator which will withstand vibration without cracking and at the same time be flexible enough to adjust itself as a permanent insulator even though the plates be expanded or twisted by heat and chemical change. My improved separator, by its permanence also aids in reducing sulphation of the grids and so supports the grid active material that the life of the whole battery is extended.

This invention also provides all of the above advantages without the introduction of complicated or expensive materials or apparatus, such as pressure vessels, ovens and the like heretofore thought necessary.

In the appended drawing—

Fig. 1 is a view of a storage battery separator core having the applicant's material and process applied thereto.

Fig. 2 is a cross-sectional view of a storage battery separator upon which the applicant's process has been practiced and showing the completed separator, certain lines having been added for purposes of description, as will appear.

Referring now to Fig. 1, G indicates generally a spray gun of the type generally well known to the art and having a removable jet piece 10, a handle 11, control valve 12, air supply pipe 14,

2

gun mixing chamber 16 and a connection 17 leading from the solution container tank 18. The internal construction and operation of such guns is well known to those skilled in this particular art and for purposes of brevity, description will be eliminated here. Suffice it to say that the air introduced through pipe 14 serves to induct and mix the solution from tank 18 through chamber 16 to nozzle 10 when valve 12 is operated. It will be appreciated that control of pressure 14 will control the speed of ejection of solution from tank 16 and the speed of solution particles in the spray 20. Through the control of such particles, it is possible to obtain a uniform pre-selected impact upon wood core 30 of the battery separator, gun G being swept from position G-1 of Fig. 2 to position G-2 so that the ridges 32 and the like of wood core 30 are coated upon all sides.

It will be understood that in the performance of my invention, I prefer to effect an immediate sealing coat over the wood core 30 and to apply thereover five or six subsequent coats whereby the coating material is thoroughly affixed, molded and bonded into an impervious film covering the wood core completely and sealing it not only against external fluids, but against the extrusion of any internal fluids or materials it may contain.

I am informed that there have been previous attempts at coating wood cores with rubber and the like by dipping and brushing certain parts thereof. However, my present process contemplates a bond between the wood fibers and the first coat and the use of vinyl chloride acetate copolymer impacted at a solution speed obtained by approximately 90 pounds air pressure at the gun nozzle and the immediate impacting and combining with the first said coating of a substantial number of coatings, all combining with and further strengthening and supplementing the original coating until it approaches a thickness of .035 inch and a weight of about 2 ounces per square foot so that the storage battery core material is enrobed in a film whose tensile strength approaches 1400 pounds per square inch but which is sufficiently flexible and elastic to allow for any movement of the wood under temperature changes while flexible and rugged enough to accommodate pressure of the storage battery plates and of irregularities in the storage battery grids without puncture.

It will thus be clear that woods heretofore unusable as storage battery separator material become usable and that acids and alkalies nor-

mally contained in such woods or which may have contaminated them in storage will no longer have any affect upon their performance as storage battery separators or upon the electrolyte components used in the operating storage battery.

What I claim is:

1. A storage battery plate separator impermeable coating of vinyl chloride acetate copolymer applied under impact and having an applied thickness of approximately thirty five one thousandths of an inch.
2. A storage battery plate separator having a wooden core completely encased in an impermeable vinyl chloride acetate copolymer film impacted in bonded layers thereover.
3. The method of processing wooden storage battery separators which comprises drying the natural wood without internal acid extraction and sealing the substantially dry wood in a non-strippable impermeable film of vinyl plastic to permanently seal the same against battery and wood acid interchange.
4. In a storage battery separator the combination of a core piece having natural acids and other materials deleterious to the usual storage battery acid action therein with an impervious plastic film bonded to the entire exterior surface of said core and encasing said natural acids and materials permanently within said core and

5 5. In a storage battery separator a wood core having six layers of vinyl chloride acetate film thereover, the first said layer impacted with said core and each succeeding layer impacted with the layer beneath so that the whole forms an impermeable heterogeneous mass.

- 10 6. In a storage battery separator, a core piece of natural untreated substantially dry wood base material encased in impacted vinyl chloride acetate copolymer plastic applied thereto by pressure impact spraying the surfaces thereof so that the 15 said core material is permanently isolated from battery action, battery fluid and reaction between its own substance, substances entrained and combined therewith and other battery components.

EDWARD CLARK.

20 References Cited in the file of this patent  
UNITED STATES PATENTS

| Number    | Name        | Date           |
|-----------|-------------|----------------|
| 2,053,058 | Wuillot     | Sept. 1, 1936  |
| 2,569,361 | Willihnganz | Sept. 25, 1951 |

FOREIGN PATENTS

| Number  | Country | Date          |
|---------|---------|---------------|
| 731,810 | France  | Sept. 8, 1932 |